

## UNITED STATES PATENT OFFICE

2,154,348

MORDANT AZO DYESTUFFS AND A PROCESS  
FOR MAKING SAMEMax Müller and Roger Ratti, Basel, Switzerland,  
assignors to the firm of Durand & Huguenin  
S. A., Basel, SwitzerlandNo Drawing. Application May 19, 1937, Serial  
No. 143,624. In Germany May 28, 1936

24 Claims. (Cl. 260—148)

This invention relates to the manufacture of valuable mordant dyeing disazo- or polyazo-dye-stuffs by coupling 2-amino-5-oxynaphthalene-7-sulphonic acid twice to produce a compound corresponding with the formula



the first coupling being in an acid medium and the second in an alkaline medium. Of the two diazo-compounds I and II indicated in the formula at least one must be derived from an ortho-aminophenol or ortho-aminonaphthol and at least one must contain the usual mordant groups such as hydroxyl and carboxyl in ortho-position to each other. These two requirements may be united in the same diazo-compound, for example the latter may be diazotized ortho-amino-salicylic acid.

The new dyestuffs are of particular value in the form of their complex metal compounds, into which they may be converted by treatment with suitable agents yielding metal in the manner now well known.

Thus for example, by the process described in British Specification No. 26460/1912, new dyestuffs may be obtained which retain the original solubility in water but contain chromium and still have the character of chrome mordant dyestuffs. According to the proportion of the chromium compound used in the production or according to the conditions of reaction the proportion of the chromium combined in the dyestuff may vary within certain limits, either all the groups present capable of being chromed or only a part thereof being saturated with chromium. Instead of chromium other trivalent metals, for instance iron, may be introduced.

If, instead of trivalent compounds, bivalent metal compounds are used in the treatment, there are produced complex metalliferous dyestuffs which are also soluble in water and have in part quite different tints from those of the parent dyestuffs. They also have the character of mordant dyestuffs and constitute a valuable addition to dyestuffs of this class.

The new dyestuffs may contain different metals simultaneously, for example a compound into which a bivalent metal has already been introduced may be converted by treatment with a

compound of a trivalent metal into water-soluble compounds which contain both the bi- and tri-valent metals in union.

All these metal compounds are suitable for all the usual methods of dyeing and printing mordant dyestuffs on various fibres, for instance cotton, artificial silk from regenerated cellulose, natural silk; in general the tints obtained are faster than those obtainable in analogous manner with the corresponding dyestuffs which have not been treated with metal.

In particular these metal compounds may be printed on the fibre in suitable manner with chromium mordants, for instance by the processes described in British Specification Nos. 15 26460/1912 and 319457, U. S. Patent No. 1,848,598, U. S. patent application Serial No. 716,001, whereby, even after a short steaming, prints are obtained of excellent fastness.

The invention is illustrated by the following examples, the parts being by weight:—

## Example 1

15.3 parts of para-aminosalicylic acid are diazotized in the usual manner and coupled in 25 acetic acid solution with 23.9 parts of 2-amino-5-hydroxynaphthalene-7-sulphonic acid. When the acid coupling is complete, the product is further coupled in alkaline solution with the diazo-solution from 23.4 parts of 1-amino-2-hydroxy-3-nitrobenzene-5-sulphonic acid. When 30 this coupling is complete, the dyestuff is salted out. It dissolves in water to a violet solution which changes towards red on addition of dilute 35 acids, becoming of lighter colour. When printed on cotton followed by a short steaming the dyestuff yields a deep-grey which on prolonged steaming becomes greenish.

When the solution of the dyestuff is heated 40 for a long time with a substance that yields chromium, for instance chromium acetate, there is obtained a complex chromium compound which may be obtained in solid form by evaporating the solution. The solution of this compound in water is blue-grey and no longer suffers change of colour on addition of acids. The new chromium compound yields when printed on cotton followed by short or long steaming a deep greenish-grey which is characterized by good fastness 45 to soaping, washing and light.

By prolonged heating with chromium lactate 50 a chromium compound is obtained which can be dyed in an acid bath on natural silk in union with a suitable chromium mordant; neutral grey 55

tints are obtained which are not varied on soaping.

If in the alkaline coupling there is used instead of the diazo-compound of 1-amino-2-hydroxy-3-nitrobenzene-5-sulphonic acid the diazo-compound of another ortho-aminophenol, for instance 1-amino-2-hydroxy-3-nitro-5-chlorobenzene or picramic acid, similar dyestuffs are obtained which also yield grey to black tints when chrome printed on cotton.

#### Example 2

23.3 parts of para-amino-ortho-sulpho-salicylic acid are diazotized in the usual manner and coupled in acetic acid solution with 23.9 parts of 2-amino-5-hydroxynaphthalene-7-sulphonic acid. The mono-azo-dyestuff thus obtained is coupled in alkaline solution with the diazo-compound of 23.4 parts of 1-amino-2-hydroxy-3-nitrobenzene-5-sulphonic acid and on completion of the coupling the new diazo-dyestuff is salted out. It dissolves in water to a red-violet solution; on adding acid to the solution the colour becomes lighter and changes towards bright-red. When printed on cotton with chromium acetate the new dyestuff yields after a short steaming a violetish-grey and on a longer steaming a somewhat greenish-grey.

By boiling the solution of the dyestuff with an agent yielding chromium, for example chromium acetate, there is obtained a complex chromium compound of the dyestuff which dissolves in water to a blueblack solution that does not suffer change of colour on addition of acid. This new chromium compound yields on cotton printing followed by short or long steaming a neutral grey-black of good fastness to soaping, washing and light.

On boiling the dyestuff with a solution of chromium lactate there is produced a chromium compound which is not suitable in this form for dyeing silk, since it separates in flocks in the dye bath. If the compound is boiled with caustic soda lye and salted out after neutralizing the lye, there is obtained a chromium compound which dyes silk in an acid bath in presence of a suitable chromium mordant. Grey-green tints are obtained which are not changed by soaping and are characterized by their good fastness to washing and to perspiration.

#### Example 3

The mono-azo-dyestuff obtainable as described in Example 2 is coupled in alkaline solution with the diazo-compound from 22.1 parts of the sodium salt of picramic acid. This disazo-dyestuff dissolves in water to a blue-red solution which becomes lighter and changes towards yellow-red on addition of acids. When chrome printed on cotton the dyestuff yields on short steaming a muddy violet, but on longer steaming a muddy violetish-grey with moderate fastness to washing with soap and a poor fastness to chlorine.

The chromium compound obtained in the usual manner yields on short or long steaming a neutral grey of good fastness to soap and washing and of rather good fastness to chlorine.

#### Example 4

15.3 parts of ortho-aminosalicylic acid are diazotized as usual and coupled in an acetic acid solution with 23.9 parts of 2-amino-5-hydroxynaphthalene-7-sulphonic acid. The mono-azo-dyestuff thus obtained is coupled in alkaline solution with the diazo-compound of 23.4 parts of 1-amino-2-hydroxy-3-nitrobenzene-5-sulphonic acid and when coupling is complete the dyestuff is salted out. It dissolves in water to a blue-red solution, changed towards violet by the addition of caustic soda lye and becoming lighter and changing towards yellow-red on the addition of acids. When chrome printed on cotton the colour is a muddy violetish-grey of poor fastness to soap, washing and chlorine after a short steaming and a greenish-grey after a longer steaming.

The chromium compound obtained in the usual manner by boiling with an agent that yields chromium dissolves in water to a grey-blue colour which is not changed either by alkali or by acid. In cotton printing the new chromium compound yields a grey-blue tint of good properties of fastness, whether the steaming be long or short.

#### Example 5

23.3 parts of ortho-amino-para-sulpho-salicylic acid are diazotized as usual and the diazo-compound is coupled in acetic acid solution with 23.9 parts of 2-amino-5-hydroxynaphthalene-7-sulphonic acid. The mono-azo-dyestuff thus obtained is coupled in alkaline solution with the diazo-compound from 22.1 parts of sodium picramate and the disazo-dyestuff is salted out when the coupling is complete. This new dyestuff dissolves in water to a bluish-red solution; on addition of acid the solution becomes lighter in colour with a change towards bright red. The dyestuff is somewhat sparingly soluble in water and yields with chromium acetate on cotton prints which are muddy blue-violet after a short steaming and violetish-black after a longer steaming; the fastness to chlorine is poor, but to washing moderately good; there is considerable loss of colour on boiling with soap.

If the solution of the dyestuff is heated with a substance that yields chromium, for instance chromium acetate, for a long time, there is obtained a chromium compound which dissolves in water to a grey-blue solution. This colour is not changed either by alkali or by acid. When printed on cotton the new chromium compound yields a greenish-grey both on short steaming and long steaming, which has good fastness to soaping, washing and chlorine and a very good fastness to light.

If a solution of chromium sulphate is used as the chroming agent there is obtained a sparingly soluble compound which dissolves when boiled with sodium carbonate to a grey-blue solution. This compound can be salted out from the solution. It has properties similar to those of the product made with the aid of chromium acetate and is also suitable for printing on cotton.

#### Example 6

The mono-azo-dyestuff obtainable as described in Example 5 is coupled in alkaline solution with the diazo-compound from 23.3 parts of ortho-amino-para-sulpho-salicylic acid. This new dyestuff dissolves in water to a red solution which becomes more blue and of deeper colour on addition of alkali. By printing on cotton with a chrome mordant muddy violet tints are obtained, whether the steaming be short or long, which are of poor fastness to chlorine and washing.

By treatment with an agent yielding chromium there is produced a complex chromium compound of the dyestuff which dissolves in water to a steel-blue solution which remains unchanged on addition of alkali or acid. In printing on cotton the chromium compound yields a neutral grey of good properties of fastness.

*Example 7*

The mono-azo-dyestuff obtainable as described in Example 5 is coupled in alkaline solution with the diazo-compound from 23.4 parts of 1-amino-2-hydroxy-3-nitrobenzene-5-sulphonic acid. This new disazo-dyestuff dissolves in water to a violet solution which becomes more blue on addition of alkali; with acids the colour becomes lighter and changes towards yellow-red. Chrome printing of the dyestuff produces muddy violetish-grey tints.

The chromium compound made in the usual manner dissolves in water to a steel-blue solution which does not change colour by addition of alkali or acid. When printed on cotton the compound yields grey-blue tints of good properties of fastness both on short and on longer steaming.

*Example 8*

23.4 parts of 1-amino-2-hydroxy-3-nitrobenzene-5-sulphonic acid are diazotized as usual and the diazo-compound is coupled in acetic acid solution with 23.9 parts of 2-amino-5-hydroxynaphthalene-7-sulphonic acid. The mono-azo-dyestuff thus produced is coupled in alkaline solution with the diazo-compound from 15.3 parts of para-amino-salicylic acid. The new disazo-dyestuff dissolves in water to a bluish-red solution. When chrome printed it yields a muddy violet tint of poor fastness to soap, chlorine and washing.

The chromium compound obtained in the usual manner dissolves in water to a blue-grey solution. When printed on cotton it yields a neutral grey of good properties of fastness.

*Example 9*

33.7 parts of 3-amino-4-sulphobenzene-azo-salicylic acid are diazotized as described in U. S. Patent No. 2,024,797 and then coupled in acetic acid solution with 23.9 parts of 2-amino-5-hydroxynaphthalene-7-sulphonic acid. The disazo-dyestuff thus obtained is coupled in alkaline

solution with the diazo-compound from 22.4 parts of 1-hydroxy-2-amino-4-chlorobenzene-6-sulphonic acid and when coupling is complete, the trisazo-dyestuff is salted out. It dissolves in water to a violetish-brown solution. When chrome printed on cotton it yields a dark-brown.

*Example 10*

The disazo-dyestuff made as described in Example 9 is coupled in alkaline solution with the diazo-compound from 23.3 parts of ortho-amino-para-sulpho-salicylic acid and when coupling is complete, the trisazo-dyestuff is salted out. The new dyestuff dissolves in water to a brown-red solution. When chrome printed on cotton it yields brown prints when the steaming is short and violetish-brown prints of poorer fastness to chlorine and washing when the steaming is long.

When treated with an agent yielding chromium the dyestuff yields a complex chromium compound which dissolves in water to a brown solution. When printed on cotton it yields a dark-brown of good properties of fastness.

When the dyestuff is treated with a copper salt, for instance by heating it with copper sulphate, there is obtained a complex copper compound which dissolves in water to a bluish-red solution. This compound yields when chrome printed on cotton or artificial silk from regenerated cellulose a reddish-brown. In like manner treatment with a nickel salt yields a complex nickel compound which when chrome printed on cotton yields a brown.

The non-metalliferous dyestuff dyes natural silk in an acid bath in presence of a suitable chromium mordant. The red-brown dyeing thus obtained may be subsequently treated on the fibre with a copper salt, whereby the fastness to light of the dyeing is essentially increased.

It is also possible in accordance with the invention to prepare a large number of other dyestuffs of which some are illustrated in the following table:

| 45 | Component coupled in—                               |                                                                         | Colour of a solution of the dyestuff in— |                             | Chromium print of the dyestuff | Colour of a solution of the chromium compound of the dyestuff in— |                             | Chrome print of the chromium compound | 45 |
|----|-----------------------------------------------------|-------------------------------------------------------------------------|------------------------------------------|-----------------------------|--------------------------------|-------------------------------------------------------------------|-----------------------------|---------------------------------------|----|
|    | 50                                                  | 50                                                                      | Water                                    | Concentrated sulphuric acid |                                | Water                                                             | Concentrated sulphuric acid |                                       |    |
| 50 | Acid medium                                         | Alkaline medium                                                         |                                          |                             |                                |                                                                   |                             |                                       | 50 |
| 50 | Orthoaminosalicylic acid.                           | 1-hydroxy-2-amino-4-chlorobenzene-6-sulphonic acid.                     | Violet.....                              | Violet.....                 | Grey-blue.....                 | Bluish grey.....                                                  | Violet.....                 | Bluish grey.                          |    |
| 55 | Do.....                                             | 1-hydroxy-2-amino-6-methyl-4-nitrobenzene.                              | do.....                                  | do.....                     | Grey.....                      | Greenish grey.....                                                | do.....                     | Greenish grey.                        | 55 |
| 55 | Do.....                                             | 1-amino-2-hydroxy-5-chloro-4-nitrobenzene.                              | Red-violet.....                          | Blue-violet.....            | Reddish-blue-grey.....         | Blue-grey.....                                                    | do.....                     | Blue-grey.                            |    |
| 55 | Do.....                                             | 5-nitro-2-aminophenol.....                                              | Violet.....                              | Violet.....                 | Grey-blue.....                 | do.....                                                           | Blue-violet.....            | Greenish-grey.                        |    |
| 60 | o-Amino-p-sulpho-salicylic acid.                    | 1-hydroxy-2-amino-4-chlorobenzene-6-sulphonic acid.                     | Blue-violet.....                         | Blue.....                   | Blue-grey.....                 | do.....                                                           | Violet.....                 | Blue-grey.                            | 60 |
| 60 | Do.....                                             | 1-hydroxy-2-amino-4-nitro-6-methylbenzene.                              | Red-violet.....                          | Blue-violet.....            | Yellowish-grey.....            | Greenish-grey.....                                                | Red-violet.....             | Grey.                                 |    |
| 60 | Do.....                                             | 1-amino-2-hydroxy-3-nitro-5-chlorobenzene.                              | Blue-violet.....                         | Blue.....                   | Blue-grey.....                 | do.....                                                           | Violet.....                 | Greenish-grey.                        | 60 |
| 65 | Do.....                                             | 1-amino-2-hydroxy-4-nitro-5-chlorobenzene.                              | Violet.....                              | Grey-blue.....              | Grey.....                      | do.....                                                           | Grey-violet.....            | Do.                                   | 65 |
| 65 | Do.....                                             | 5-nitro-2-aminophenol.....                                              | Reddish-blue.....                        | do.....                     | Greenish-grey.....             | do.....                                                           | do.....                     | do.                                   |    |
| 65 | Do.....                                             | 1-hydroxy-2-amino-4-methyl-6-nitrobenzene.                              | do.....                                  | Blue-violet.....            | Grey.....                      | Grey-blue.....                                                    | M u d d y violet.....       | Grey.                                 |    |
| 65 | Do.....                                             | 1-hydroxy-2-amino-4-nitrobenzene-6-sulphonic acid. Picraminic acid..... | Red.....                                 | Dark-violet.....            | Grey-black.....                | do.....                                                           | Dark-violet.....            | Greenish-grey.                        |    |
| 70 | o-Amino-p-chloro-salicylic acid.                    | Picraminic acid.....                                                    | do.....                                  | Blue-violet.....            | M u d d y grey-violet.....     | do.....                                                           | Violet.....                 | Do.                                   | 70 |
| 70 | 1-hydroxy-2-amino-6-nitrobenzene-4-sulphonic acid.  | o-Amino-p-sulphosalicylic acid.                                         | Red-violet.....                          | Brown-violet.....           | Blue-grey.....                 | Blue.....                                                         | do.....                     | do.                                   |    |
| 70 | 1-hydroxy-2-amino-4-chlorobenzene-6-sulphonic acid. | do.....                                                                 | do.....                                  | Red-violet.....             | Violet.....                    | Blue-violet.....                                                  | Blue-violet.....            | Bluish grey.                          |    |

Similar dyestuffs may be obtained according to the present process by using ortho-amino-naphthol-compounds instead of ortho-amino-phenol-compounds.

5 What we claim is:—

1. A process of preparing mordant polyazo-dyestuffs and water soluble metal compounds thereof, comprising coupling 2-amino-5-hydroxynaphthalene-7-sulphonic acid twice, a first time 10 in a weak acid medium with a diazo-compound I and a second time in an alkaline medium with a diazo-compound II, to produce a dyestuff of the general type:

15



20

the two diazo-compounds I and II being derived from an aromatic ortho-hydroxy-amine and at least one of them having a hydroxy group and a carboxyl group in ortho-position to one another, and treating the dyestuff thus obtained with metal yielding agents.

2. A process of preparing mordant polyazo-dyestuffs and water soluble metal compounds thereof, comprising coupling 2-amino-5-hydroxynaphthalene-7-sulphonic acid twice, a first time in a weak acid medium with a diazo-compound I and a second time in an alkaline medium with a diazo-compound II, to produce a dyestuff of the general type:

25



30

the two diazo-compounds I and II being derived from an aromatic ortho-hydroxy-amine and both of them having a carboxyl group in ortho-position to a hydroxy group, and treating the dyestuffs thus obtained with metal yielding agents.

3. A process of preparing mordant polyazo-dyestuffs and water soluble metal compounds thereof, comprising coupling 2-amino-5-hydroxynaphthalene-7-sulphonic acid twice, a first time in a weak acid medium with a diazo-compound I and a second time in an alkaline medium with a diazo-compound II, to produce a dyestuff of the general type:

35



40

the two diazo-compounds I and II being derived from an ortho-amino-phenol-compound and at least one of them having a hydroxy group and a carboxyl group in ortho-position to one another, and treating the dyestuff thus obtained with metal yielding agents.

4. A process of preparing mordant polyazo-dyestuffs and water soluble metal compounds thereof, comprising coupling 2-amino-5-hydroxynaphthalene-7-sulphonic acid twice, a first time in a weak acid medium with a diazo-compound I and a second time in an alkaline medium with

a diazo-compound II, to produce a dyestuff of the general type:



5

the two diazo-compounds I and II being derived from an ortho-amino-phenol-compound and both of them having a carboxyl group in ortho-position to a hydroxy group, and treating the dyestuff thus obtained with metal yielding agents.

5. A process of preparing mordant polyazo-dyestuffs and water soluble metal compounds thereof, comprising coupling 2-amino-5-hydroxynaphthalene-7-sulphonic acid twice, a first time in a weak acid medium with a diazotized ortho-amino-salicylic-acid-compound and a second time in an alkaline medium with a diazotized ortho-amino-phenol-compound, and treating the dyestuff thus obtained with metal yielding agents.

6. A process of preparing mordant polyazo-dyestuffs and water soluble metal compounds thereof, comprising coupling 2-amino-5-hydroxynaphthalene-7-sulphonic acid twice, a first time in a weak acid medium with diazotized ortho-amino-para-sulphosalicylic acid and a second time in an alkaline medium with a diazotized ortho-amino-phenol-compound, and treating the dyestuff thus obtained with metal yielding agents.

7. A process of preparing mordant polyazo-dyestuff and water soluble metal compounds thereof, comprising coupling 2-amino-5-hydroxynaphthalene-7-sulphonic acid twice, a first time in a weak acid medium with a diazotized ortho-amino-salicylic-acid-compound and a second time in an alkaline medium with a diazotized ortho-amino-salicylic-acid-compound, and treating the dyestuff thus obtained with metal yielding agents.

8. A process of preparing mordant polyazo-dyestuffs and water soluble metal compounds thereof, comprising coupling 2-amino-5-hydroxynaphthalene-7-sulphonic acid twice, a first time in a weak acid medium with diazotized ortho-amino-para-sulphosalicylic acid and a second time in an alkaline medium with diazotized ortho-amino-para-sulphosalicylic acid, and treating the dyestuff thus obtained with metal yielding agents.

9. A process of preparing mordant polyazo-dyestuffs and water soluble metal compounds thereof, comprising coupling 2-amino-5-hydroxynaphthalene-7-sulphonic acid twice, a first time in a weak acid medium with a diazo-compound I and a second time in an alkaline medium with a diazo-compound II, to produce a dyestuff of the general type:



60

the two diazo-compounds I and II being derived from an aromatic ortho-hydroxy-amine and at least one of them having a hydroxy group and a carboxyl group in ortho-position to one another, and treating the dyestuff thus obtained with an agent yielding a bivalent metal.

10. A process of preparing mordant polyazo-dyestuffs and water soluble metal compounds thereof, comprising coupling 2-amino-5-hydroxynaphthalene-7-sulphonic acid twice, a first time in a weak acid medium with a diazo-compound I and a second time in an alkaline medium with

75

naphthalene-7-sulphonic acid twice, a first time in a weak acid medium with a diazo-compound I and a second time in an alkaline medium with a diazo-compound II, to produce a dyestuff of the general type:



the two diazo-compounds I and II being derived from an aromatic ortho-hydroxy-amine and at least one of them having a hydroxy group and a carboxyl group in ortho-position to one another, and treating the dyestuff thus obtained with a copper yielding agent.

11. A process of preparing mordant polyazo-dyestuffs and water soluble metal compounds thereof, comprising coupling 2-amino-5-hydroxynaphthalene-7-sulphonic acid twice, a first time in a weak acid medium with a diazo-compound I and a second time in an alkaline medium with a diazo-compound II, to produce a dyestuff of the general type:



35 the two diazo-compounds I and II being derived from an aromatic ortho-hydroxy-amine and at least one of them having a hydroxy group and a carboxyl group in ortho-position to one another, and treating the dyestuff thus obtained with copper sulphate.

40 12. A process of preparing mordant poly-azo-dyestuffs and water soluble metal compounds thereof, comprising coupling 2-amino-5-hydroxynaphthalene-7-sulphonic acid twice, a first time in a weak acid medium with a diazo-compound I and a second time in an alkaline medium with a diazo-compound II, to produce a dyestuff of the general type:



55 the two diazo-compounds I and II being derived from an aromatic ortho-hydroxy-amine and at least one of them having a hydroxy group and a carboxyl group in ortho-position to one another, and treating the dyestuff thus obtained with an agent yielding a trivalent metal.

60 13. A process of preparing mordant polyazo-dyestuffs and water soluble metal compounds thereof, comprising coupling 2-amino-5-hydroxynaphthalene-7-sulphonic acid twice, a first time in a weak acid medium with a diazo-compound I and a second time in an alkaline medium with a diazo-compound II, to produce a dyestuff of the general type:



65 the two diazo-compounds I and II being derived from an aromatic ortho-hydroxy-amine and at least one of them having a hydroxy group and a carboxyl group in ortho-position to one another, and treating the dyestuff thus obtained with a chromium yielding agent.

14. A process of preparing mordant polyazo-dyestuffs and water soluble metal compounds thereof, comprising in coupling 2-amino-5-hydroxynaphthalene-7-sulphonic acid twice, a first time in a weak acid medium with a diazo-compound I and a second time in an alkaline medium with a diazo-compound II, to produce a dyestuff of the general type:



20 the two diazo-compounds I and II being derived from an aromatic ortho-hydroxy-amine and at least one of them having a hydroxy group and a carboxyl group in ortho-position to one another, and treating the dyestuff thus obtained with chromium acetate.

25 15. A process of preparing mordant polyazo-dyestuffs and water soluble metal compounds thereof, comprising coupling 2-amino-5-hydroxynaphthalene-7-sulphonic acid twice, a first time in a weak acid medium with a diazo-compound I and a second time in an alkaline medium with a diazo-compound II, to produce a dyestuff of the general type:



35 the two diazo-compounds I and II being derived from an aromatic ortho-hydroxy-amine and at least one of them having a hydroxy group and a carboxyl group in ortho-position to one another, and treating the dyestuff thus obtained with a bivalent and a trivalent metal yielding agent.

40 16. A process of preparing mordant disazo-dyestuffs and water soluble metal compounds thereof, comprising coupling 2-amino-5-hydroxynaphthalene-7-sulphonic acid twice, a first time in a weak acid medium with a diazotized ortho-amino-salicylic-acid-compound and a second time in an alkaline medium with a diazotized ortho-amino-phenol compound, and treating the dyestuff thus obtained with a copper yielding agent.

45 17. A process of preparing a mordant disazo-dyestuff and a water soluble metal compound thereof, comprising coupling 2-amino-5-hydroxynaphthalene-7-sulphonic acid twice, a first time in a weak acid medium with diazotized ortho-amino-para-sulphosalicylic acid and a second time in an alkaline medium with diazotized 1-amino-2-hydroxy-5-chloro-3-sulphonic acid, and treating the dyestuff thus obtained with copper sulphate.

50 18. A process of preparing mordant disazo-dyestuffs and water soluble metal compounds thereof, comprising coupling 2-amino-5-hydroxynaphthalene-7-sulphonic acid twice, a first time in a weak acid medium with a diazotized ortho-amino-salicylic acid compound and a second

time in an alkaline medium with a diazotized ortho-aminophenol compound, and treating the dyestuff thus obtained with a chromium yielding agent.

- 5 19. A process of preparing a mordant disazo-dyestuff and a water soluble metal compound thereof, comprising coupling 2-amino-5-hydroxynaphthalene-7-sulphonic acid twice, a first time in a weak acid medium with diazotized ortho-10 amino-para-sulphosalicylic acid and a second time in an alkaline medium with diazotized 1-amino-2-hydroxy-5-nitrobenzene-3-sulphonic acid and treating the dyestuff thus obtained with chromium acetate.

- 15 20. Water soluble metal compounds of polyazo-dyestuffs corresponding to the following general formula:



- 25 25 wherein the two aromatic radicals R<sub>1</sub> and R<sub>2</sub> bear a hydroxy group in ortho-position to the azo-groups and at least one of them has a carboxyl group in ortho-position to a hydroxy group, these dyestuffs containing at least one metal in complex 30 combination.

21. Water soluble metal compounds of polyazo-dyestuffs corresponding to the following general formula:



- 40 40 wherein the two aromatic radicals R<sub>1</sub> and R<sub>2</sub> bear

a hydroxy group in ortho-position to the azo-groups and at least one of them has a carboxyl group in ortho-position to a hydroxy group, these dyestuffs containing copper in complex 5 combination.

22. Water soluble metal compounds of polyazo-dyestuffs corresponding to the following general formula:



15 wherein the two aromatic radicals R<sub>1</sub> and R<sub>2</sub> bear a hydroxy group in ortho-position to the azo-groups and at least one of them has a carboxyl group in ortho-position to a hydroxy group, these dyestuffs containing chromium in complex 20 combination.

- 25 23. The new water soluble cupriferous disazo-dyestuff, obtained by coupling 2-amino-5-hydroxynaphthalene-7-sulphonic acid twice, a first time in a weak acid medium with diazotized ortho-amino-para-sulphosalicylic acid and a second time in an alkaline medium with diazotized 1-amino-2-hydroxy-5-chloro-3-sulphonic acid and treating the dyestuff thus obtained with a 30 copper yielding agent.

- 35 24. The new water soluble chromiferous disazo-dyestuff, obtained by coupling 2-amino-5-hydroxynaphthalene-7-sulphonic acid twice, a first time in a weak acid medium with diazotized ortho-amino-para-sulphosalicylic acid and a second time in an alkaline medium with diazotized 1-amino-2-hydroxy-5-nitrobenzene-3-sulphonic acid and treating the dyestuff thus obtained with a chromium yielding agent.

MAX MÜLLER. 40  
ROGER RATTI.